# EUROPEAN PATENT SPECIFICATION

(11) **EP 1 137 719 B1**
(45) Date of publication and mention of the grant of the patent: **22.02.2006**
(21) Application number: 99962630.2
(22) Date of filing: 23.11.1999
(51) Int. Cl.: C09C 3/10, D21H 11/20, D21H 17/69

(54) **METHOD OF PRODUCING A FIBER OR GROUP OF FIBERS HAVING A COATING OF POLYMERS INTERACTING WITH EACH OTHER**
VERFAHREN ZUR HERSTELLUNG VON FASERN ODER GRUPPEN VON FASERN DIE MIT POLYMEREN BESCHICHTEN SIND, DIE UNTEREINANDER WECHSELWIRKEN.
PROCEDE DE FABRICATION D'UNE FIBRE OU D'UN GROUPE DE FIBRES COMPORTANT UN REVETEMENT DE POLYMERES EN INTERACTION LES UNS AVEC LES AUTRES

(30) Priority: 30.11.1998 SE 9804123
(43) Date of publication of application: 04.10.2001
(73) Proprietor: SCA Hygiene Products AB, 405 03 Göteborg (SE)
(72) Inventor: FORSBERG, Sven, S-856 31 Sundsvall (SE); WAGBERG, Lars, S-854 60 Sundsvall (SE)
(74) Representative: Egeröd, Lisbeth
(86) International application number: PCT/SE1999/002149
(87) International publication number: WO 2000/032702

(56) References cited:
- EP-A2- 0 850 879
- WO-A1-95/32335
- DE-A1- 2 516 097
- US-A- 4 495 245
- US-A- 4 925 530
- US-A- 5 208 111
- US-A- 5 244 542

## Description

### Technical field

The present invention refers to a method of producing a fiber or group of fibers having a coating of at least two, preferably at least three, outside each other located thin layers of interacting polymers, at which the fiber or group of fibers is treated in consecutive steps with solutions of the interacting polymers. Such a coating modifies the properties of the fibers as well as the properties of the products, e g paper and nonwoven, in which the treated fibers are contained.

### Background of the invention

The increased use of recovered fibers in paper production and the use of components with poorer bonding properties, such as mineral fillers, have increased the need for more effective dry strength agents in the paper. Traditionally two different methods have been used for adding strength improving chemicals to the paper, viz. by adding chemicals at the wet end of the paper process or by surface application by means of a size press. Wet end addition is usually more effective than surface application counted per kg utilized product. In order to maintain the addition made in the wet end in the paper sheet, wet end chemicals are mainly exclusively cationic, and for making them less sensitive to dissolved and colloidal materials and the increased concentration of electrolytes caused by the increased closing of the systems, their cationic charge is usually increased. This leads in turn to a decreased saturation adsorption of the additive chemicals to the fibers, which leads to a reduced maximum effect of the additive chemicals. This involves that there is a need both for new methods of applying strength-improving chemicals to the paper, and new chemical systems.

Besides there is an increased need for improving the opacity of the finished paper. Since the today most frequently used strength agents contribute negatively to the opacity the need for new methods of developing strength in the paper is further reinforced.

Such a way would be to utilize size presses to a higher extent, but this would however lead to large reductions of the manufacturing capacity and the production economy since the paper has to be dried once further depending on the rewet it is exerted to in the size press.

This involves that there is a great need for new ways of treating fibers, in the wet end of the paper machine.

Also treatment with a similar process such as size presses may be of interest if the quality of the produced paper is herewith increased in a satisfactory way, so that the above mentioned drawbacks will be of less importance.

It is known to build up thin multilayers of electro active polymers on an electrostatically charged substrate for use in optics, such as sensors, friction reduction etc. This is described in for example in *Thin Solid Films, 210*/*211 (1992) 831-835* and in *Thin Solid Films, 244 (1994) 806-809*. The substrate is herewith immersed alternatingly in diluted solutions of a polycation with an intermediate rinsing in order to remove rests of the previous polyion which is not bonded to the substrate. The thickness of each deposited layer is described to be between 5-20Å. There is no indication that the treated substrates could be particles, such as fibers.

In US 5,338,407 there is disclosed a method for improving the dry strength properties of paper, at which an anionic carboxy methyl guar or carboxy methyl hydroxy ethyl guar and a cationic guar is added to the furnish. These two components are either added in mixture or separately. There is no indication that the treatment is made under such conditions that a double layer is built up on the fibers with one component in one layer and the other component in the other layer.

In the US patents 5,507,914 and 5,185, 062 there are disclosed methods for improving the dewatering properties and the retention of paper by adding anionic and cationic polymers to the pulp. There is no indication that the treatment takes place under such conditions that a double- or multilayer is created on the pulp fibers with the anionic component in one layer and the cationic component in the other layer.

Dual surface treatment of filler particles with anionic and cationic polymers is disclosed in EP-A-0 850 879, WO 95/32335, US-A-4,495,245 and US-A-4,925,530. There is no indication that the treatment takes place under such controlled conditions that a double- or multilayer is created on the pulp fibers with the anionic component in one layer and the cationic component in the other layer.

### The object and most important features of the invention

The object of the present invention is to provide a method for producing fibers or groups of fibers, having a coating of at least two, preferably at least three, outside each other located thin layers of interacting polymers, at which the fiber or group of fibers is treated in consecutive steps with solutions of the interacting polymers. This has been provided by the fact that excess of the previous polymer is removed between each treatment step alternatively that the respective polymer is added only in such an amount in each step that substantially all polymer is adsorbed to the fiber surface.

The fibers or groups of fibers may be of optional type, however e g cellulosic fibers, regenerated fibers and different types of synthetic fibers are mainly concerned.

The interacting polymers are preferably alternating cationic and anionic polyelectrolytes, but they may also be so called zwitter ions.

The thickness of each of said thin layers is preferably between 3 and 100Å, more preferably between 7 and 20Å.

The invention further refers to a paper- or nonwoven product, which contains fibers produced by the method described above.

### Description of drawings

Fig. 1 shows in the form of bar charts the tensile strength index of sheets made of cellulosic fibers with different numbers of applied polymer layers.
Fig. 2 shows in the form of a bar chart the increase of tensile strength of paper containing pulp fibers coated with an anionic and a cationic polymer added at the same time and added separately in six consecutive steps rinsing away the excess of polymer between each step.

### Description of the invention

According to the present invention fibers or groups of fibers, are treated with interacting polymers in order to build up thin multilayers of the interacting polymers on the fiber surface. In principle the technique described in for example above mentioned articles from *Thin Solid Films* is used in case alternating cationic and anionic polyelectrolytes are used as interacting polymers, with the difference that according to the invention the substrate is fibers groups of fibers.

The fibers are treated in consecutive steps with solutions of the interacting polymers, at which the treatment time for each step is sufficient for forming a layer of the desired molecular thickness, preferably of the magnitude 5-100Å. The interaction between the fibers can be in the form of electrostatic forces, at which the polymers consist of alternating cationic and anionic polyelectrolytes, or by interaction between nonionic polymers by means of e g dispersion forces or hydrogen bonds. Examples of this type of interaction between nonionic polymers are adsorption of polyethylene oxide on unbleached cellulosic fibers and complex formation between polyethylene oxide and polyacrylic acid.

In case the interacting polymers are alternating cationic and anionic polyelectrolytes the first layer should be a cationic polymer for particles or groups of particles having an anionic surface, which for example is the case for cellulosic fibers, and vice versa. Possible excess of the previous polyelectrolyte can be removed between every treatment step, e g by rinsing with water. Alternatively the addition is controlled in such a way that no excess amount of the respective polymer is added in each step, so that substantially all polymer is adsorbed to the fiber surface.

The method is based on electrostatic attraction between oppositely charged polyelectrolytes for building the desired multilayers. By treating the fibers in consecutive steps with a solution containing polyions of opposite charge and pennit these spontaneously to adsorb to the particle surface, multilayers of the stated kind are built up. In principle all types of polyelectrolytes may be used.

Through such a treatment of fibers or groups of fibers, it is possible to make new types of surface modifications to them. By for example treating fibers with consecutive layers of hydrophobic, charged polyelectrolytes it would be possible for example to develop new types of hydrophobizing chemicals for the hydrophobization of paper. It would also be possible to build up "intelligent" surface layers on fibers, which alter the properties with temperature, pH, salt content etc. These changes could for example be based on fundamental knowledge about modem theories on interaction between polymers and surfactants.

Further applications are ion-exchanging fibers where "membranes" with ion-exchanging properties are provided on the fiber surface, wet strength agents where the added polymers are reactive with the fibers and with each other, in order to provide permanent bonds between the fibers and for the production of highly swelling surface layers, where the added chemicals form swollen gel structures on the fiber surface for use in absorbent hygiene products. Another possible application are new types of fibers for printing paper, where the adsorbed polymers change colour when they are exerted to an electric, magnetic or electromagnetic field. Such polymers are available today.

The fibers that are treated with the method according to the invention can be of optional kind, natural as well as synthetic fibers. Mainly cellulosic fiber are concerned. However it would be possible to treat synthetic fibers, for example for giving them a more hydrophilic surface.

Also groups of fibers can be treated according to the method.

Examples of suitable anionic and cationic polyelectrolytes which may be used in the method according to the invention are given below.
*Anionic polyelectrolytes:* Anionic starch with different degrees of substitution, polystyrene sulphonate, carboxy methyl cellulose with different degrees of substitution, anionic galactoglucomannan, polyphosphoric acid, polymethacrylic acid, polyvinyl sulphate, alginate, copolymers of acryl amide and acrylic acid or 2-acrylic amide-2-alkylpropane sulphonic acid.

*Cationic polyelectrolyte:* Cationic galactoglucomannan, polyvinyl amine, polyvinyl pyridine and its N-alkyl derivatives, polyvinyl pyrrolidone, chitosan, alginate, modified polyacryl amides, polydiallyl dialkyl, cationic amide amines, condensation products between dicyane diamides, formaldehyde and an ammonium salt, reaction products between epichlorhydrine, polyepichlorhydrine and ammonia, primary and secondary amines, polymers formed by reaction between ditertiary amines or secondary amines or dihaloalkanes, polyethylene imines and polymers formed by polymerisation ofN-(dialkylaminoalkyl)acrylic amide monomers.

### Example 1

The example below shows the increase of tensile strength of sheets made in a dynamic sheet former. The pulp that is used was bleached SWK (softwood sulphate pulp) beaten in accordance with SCAN-C 18:65, diluted to 3g/l and pH adjusted to 8. PVAm (polyvinyl amine), a cationic polymer, was added in excess and was given time to react after which the excess of polymer was washed away from the fiber suspension by means of water. After that CMC (carboxy methyl cellulose), an anionic polymer, was added in excess, and after 10 minutes non-adsorbed polymer was removed through washing. Admixture of PVAm and CMC was repeated in several steps. After each addition of CMC the so called dynamic sheet former was used for making sheets having a basis weight of 80 g/m². The sheets were tested with respect to tensile strength according to SCAN-P 67:93. The results are shown in Table 1 below and proves clearly an improvement of tensile strength index with the number of applied polymer layers.

**Table 1**

| Polymer layer (P=PVAm, C=CMC) | Tensile strength index (kNm/kg) |
|---|---|
| No polymer | 39,0 |
| P | 53,6 |
| PC | 56,6 |
| PCPC | 69,4 |
| PCPCPC | 75,8 |

The results are also shown in Fig. 1 in the drawings.

### Example 2

Two types of polymers were used: an anionic polyacryl amide (A-PAM), Percol 155 from Ciba, and a canonic polydimethyl diallyl ammonium chloride (DMDAAC) also from Ciba. The pulp that was used was unrefined, fully bleached longfiber pulp, pH 8 in all tests. The dosing of the polymers were done in two different ways:
A) all at the same time and in this case 3.9 kg/ton A-PAM was added first and then 6.6 kg/ton polyDMDAAC was added.
B) Six layers of 1.1 kg/ton polyDMDAAC and 0.65 kg/ton A-PAM in the respective layers were added. Excess of polymer was removed between the dosings.

Handsheets were then made and the strength (tensile strength index) was measured. In Fig. 2 the strength increase in % is shown for the two different cases. As can clearly be seen it is much more effective to add the polymers in layers in a controlled manner.

## Claims

1. Method of producing a fiber or group of fibers having a coating of at least two, preferably at least three, outside each other located thin layers of Interacting polymers, at which the fiber or group of fibers is treated in consecutive steps with solutions of the interacting polymers,
**characterized in**
**that** excess of the previous polymer is removed between each treatment step alternatively that the respective polymer is added only in such an amount in each step that substantially all polymer is adsorbed to the fiber surface.

2. Method as claimed in claim 1,
**characterized in**
**that** the fiber is a cellulosic fiber.

3. Method as claimed In claim 1,
**characterized in**
**that** the fiber is a synthetic or regenerated fiber.

4. Method as claimed in any of the preceding claims,
**characterized in**
**that** the interacting polymers are alternating cationic and anionic polyelectrolytes or ampholytes.

5. Method as claimed in any of the preceding claims,
**characterized in**
**that** each of said thin layers has a thickness of between 1 and 100Å.

6. Method as claimed in any of the preceding claims,
**characterized in**
**that** each of said thin layers has a thickness between 7 and 20Å.

7. Paper or nonwoven product,
**characterized in**
**that** it contains fibers produced according to the method of any of claims 1-6.

## Patentansprüche

1. Verfahren zur Herstellung einer Faser oder einer Gruppe von Fasern, die eine Beschichtung von mindestens zwei, vorzugsweise mindestens drei, ausserhalb voneinander gelegenen dünnen Schichten wechselwirkender Polymere aufweist, worin die Faser oder die Gruppe von Fasern in aufeinanderfolgenden Schritten mit Lösungen der wechselwirkenden Polymere behandelt ist, **dadurch gekennzeichnet, dass** der Überschuas des vorherigen Polymers zwischen jedem Behandlungsschritt entfernt wird, alternativ, dass das jeweilige Polymer nur in einer solchen Menge in jedem Schritt zugegeben wird, dass im wesentlichen das ganze Polymer auf der Faseroberfläche adsorbiert wird.

2. verfahren gemäss Anspruch 1, **dadurch gekennzeichnet, dass** die Faser eine cellulosische Faser ist.

3. Verfahren gemäss Anspruch 1, **dadurch gekennzeichnet, dass** die Faser eine synthetische oder regenerierte Faser ist.

4. verfahren gemäss einem der vorangehenden Ansprüche, **dadurch gekennzeichnet, dass** die wechselwirkenden Polymere alternierende kationische und anionische Polyelektrolyte oder Ampholyte sind.

5. Verfahren gemäss einem der vorangehenden Ansprüche, **dadurch gekennzeichnet, dass** jede der dünnen Schichten eine Dicke zwischen 1 und 100 Å aufweist.

6. Verfahren gemäss einem der vorangehenden Ansprüche, **dadurch gekennzeichnet, dass** jede der dünnen Schichten eine Dicke zwischen 7 und 20 Å aufweist.

7. Papier oder Vliesprodukt, **dadurch gekennzeichnet, dass** es Fasern enthält, die gemäss dem Verfahren von irgendeinem der Ansprüche 1 bis 6 hergestellt wurden.

## Revendications

1. Procédé de production d'une fibre ou d'un ensemble de fibres, dotée(s) d'un revêtement constitué d'au moins deux, et de préférence, d'au moins trois minces couches de polymères interagissants, disposées à l'extérieur l'une de l'autre, dans lequel procédé l'on traite la fibre ou l'ensemble de fibres, au cours d'étapes successives, avec des solutions des polymères interagissants,
**caractérisé en ce que**, à chaque intervalle entre deux étapes de traitement, on élimine l'excès du polymère de l'étape précédente, ou autrement, **en ce que**, à chaque étape, l'on n'ajoute du polymère concerné qu'en une quantité telle que pratiquement la totalité de ce polymère s'adsorbe à la surface de la fibre.

2. Procédé conforme à la revendication 1, **caractérisé en ce que** la fibre est une fibre cellulosique.

3. Procédé conforme à la revendication 1, **caractérisé en ce que** la fibre est une fibre synthétique ou une fibre régénérée.

4. Procédé conforme à l'une des revendications précédentes, **caractérisé en ce que** les polymères interagissants sont des ampholytes ou des polyélectrolytes anioniques et cationiques alternants.

5. Procédé conforme à l'une des revendications précédentes, **caractérisé en ce que** chacune desdites minces couches est épaisse de 1 à 100 Å.

6. Procédé conforme à l'une des revendications précédentes, **caractérisé en ce que** chacune desdites minces couches est épaisse de 7 à 20 Å.

7. Papier ou produit non-tissé, **caractérisé en ce qu'**il contient des fibres produites par un procédé conforme à l'une des revendications 1 à 6.
